

Patented Dec. 11, 1928.

1,694,879

# UNITED STATES PATENT OFFICE.

STEWART S. KURTZ, JR., OF AKRON, OHIO, ASSIGNOR TO THE GOODYEAR TIRE & RUBBER COMPANY, OF AKRON, OHIO, A CORPORATION OF OHIO.

## METHOD OF TREATING AIR BAGS.

No Drawing.

Application filed November 21, 1927. Serial No. 234,924.

My invention relates to methods of preserving the interior surfaces of airbags and it has, for its primary object, the provision of a material which, when introduced into an 5 airbag, forms a permanent coating over the exposed surfaces.

More specifically, my invention has, for one of its objects, the provision of a material which, when spread over the inner 10 surface of an airbag, tends to absorb oxygen and thus to become relatively thick and viscous so that it will not flow.

It has been observed that glycerine solutions injected into airbags used as 15 expandable cores during the vulcanization of pneumatic tires, tend to collect in the lower portions of the bags, thus leaving the upper surfaces exposed to the action of oxygen, which attacks the rubber, rendering it brittle and 20 thus causing cracking.

In a copending application of Cornelis Van Rennes, Serial No. 239,127, filed December 10, 1927, is disclosed a method of forming a protective coating material which, when 25 injected into an airbag, will remain uniformly spread over the inner surface thereof. This object is accomplished by employing a glycerine solution containing a material, such as an inert pigment, adapted to cause it to become 30 thick and relatively viscous.

I have discovered that drying oils are particularly adapted for this purpose. These oils may readily be incorporated into the glycerine by employing a suitable emulsifying 35 agent, such as soap and a stabilizing ingredient, such as glue. The drying oils that absorb oxygen from the air, become relatively viscous and thus impart a considerable degree of viscosity to the glycerine solution to 40 which they are added. Rape seed oil is a very satisfactory drying oil for this purpose. However, linseed oil, cotton seed oil and other unsaturated hydrocarbons, known as drying oils, may also be employed as substitutes 45 therefor. The following is an example of a formula for a compound which gives very excellent results.

Prepare a glue dispersion consisting of 1 part of glue and  $1\frac{1}{2}$  parts of water. Also 50 prepare a 16% solution of soap. Intermix one volume of a glue dispersion with one volume of glycerine and .2 of a volume of soap solution. Heat these materials and then add, with vigorous agitation, one volume of rape

seed oil. Introduce the emulsion thus formed 55 into the bag while yet hot, and rotate and invert the bag in order to distribute the materials over the interior thereof while they are still relatively fluid. These materials soon absorb oxygen from the air in the bag and 60 thus become so thick and viscous that they will not flow readily even when subjected to the relatively high temperature required to vulcanize a tire.

The solution may be introduced into the 65 bags either before or after they are vulcanized, but it is preferable to introduce it before, because it permits the use of air as an inflating gas during the vulcanization of the 70 bag instead of carbon dioxide, which is usually employed because of its low chemical reactivity.

It will be apparent from the previous discussion of my invention that I have discovered a coating material which is adapted to 75 form a very permanent coating over the interior surfaces of an airbag or other rubber surface that is exposed to the action of oxygen. This material is relatively inexpensive 80 and may be prepared with ease.

While I have disclosed only the preferred 85 embodiments of my invention and described those embodiments in detail, it will be apparent to those skilled in the art that the invention is not so limited, but that various modifications may be made therein without departing from the spirit of the invention or from the scope of the appended claims.

### What I claim is:

1. A method of preserving the interior surfaces of airbags which comprises introducing into the bag a solution containing glycerine and a drying oil. 90

2. A method of preserving the interior surfaces of airbags which comprises introducing 95 into the bags a solution containing glycerine, a drying oil and an emulsifying agent.

3. A method of preserving the interior surfaces of airbags which comprises introducing 100 into the bag a solution containing glycerine, a drying oil, an emulsifying agent and a stabilizing ingredient.

4. A method of preserving the interior surfaces of airbags which comprises introducing 105 into the bags an emulsion composed of glycerine, a drying oil, an emulsifying agent and a stabilizing ingredient.

5. A method of preserving airbags which

comprises introducing into the bags a solution containing a drying oil, an emulsifying agent and a stabilizing ingredient.

6. A method of preserving the interior surfaces of airbags which comprises introducing into the bags a solution composed of glycerine and rape seed oil.

7. A method of preserving the interior surfaces of airbags which comprises introducing into the bags a solution of glycerine, rape seed oil and an emulsifying agent.

8. A method of preserving the interior surfaces of airbags which comprises intro-

ducing into the bags a solution of glycerine, rape seed oil, an emulsifying agent and a stabilizing ingredient.

9. A method of preserving the interior surfaces of airbags which comprises introducing into the bags a solution of glycerine, rape seed oil, glue and soap.

In witness whereof, I have hereunto signed my name.

Signed at Akron, in the county of Summit, and State of Ohio, this 19th day of November, 1927.

STEWART S. KURTZ, JR.